

## [54] STABILIZATION OF MERCURY-VAPOR DISCHARGE LAMPS

[75] Inventors: Charles E. Beck, Chesterland; D. Richard Zatyko, Richmond Heights, both of Ohio

[73] Assignee: General Electric Company, Schenectady, N.Y.

[22] Filed: May 10, 1972

[21] Appl. No.: 252,341

[52] U.S. Cl. .... 313/44, 313/34

[51] Int. Cl. .... H01j 9/44

[58] Field of Search ..... 313/34, 44, 109, 174; 315/112

## [56] References Cited

## UNITED STATES PATENTS

|           |         |                 |                 |
|-----------|---------|-----------------|-----------------|
| 2,966,602 | 12/1960 | Waymouth et al. | ..... 313/44 X  |
| 3,205,394 | 9/1965  | Ray             | ..... 313/109   |
| 3,284,664 | 11/1966 | Morin et al.    | ..... 313/109 X |
| 3,331,977 | 7/1967  | Wainio          | ..... 313/34    |
| 3,339,100 | 8/1967  | Menelly         | ..... 313/174 X |

## OTHER PUBLICATIONS

Underwood et al., "External Control of Mercury Pres-

sure of Fluorescent Lamps" Illuminating Engineering, Vol. LV, No. 1, January, 1960, pp. 47-55

Beck et al., "Light Output of 1.5 Ampere Fluorescent Lamp Designs" Illuminating Engineering, Vol. LXIII, No. 4, April, 1968, pp. 167-175

Primary Examiner—Herman Karl Saalbach

Assistant Examiner—Richard A. Rosenberger

Attorney, Agent, or Firm—Norman C. Fulmer; Henry P. Truesdell; Frank L. Neuhauser

## [57] ABSTRACT

A method for prestabilizing mercury-vapor discharge lamps, such as fluorescent lamps. After lamp assembly, the lamp is temporarily operated while at the same time cooling, to a temperature lower than its normal intended operating temperature, a small area of the bulb, at the normal "cold spot" location where the mercury will condense during lamp operation. This causes the mercury to quickly condense and adhere to the phosphor and bulb at the cold spot. The lamp may then be shipped and put into use without the need for any appreciable further stabilization.

5 Claims, 4 Drawing Figures



PATENTED JUN 28 1974

3,821,578

FIG. 2.



FIG. 1. (PRIOR ART)



FIG. 3.



FIG. 4.



## STABILIZATION OF MERCURY-VAPOR DISCHARGE LAMPS

### BACKGROUND OF THE INVENTION

The invention is in the field of mercury-vapor discharge lamps, such as fluorescent lamps, and more specifically relates to the stabilization of the mercury pressure in such lamps.

When a mercury-vapor discharge lamp is first operated, it goes through a period of "unstabilized" operation, accompanied by reduced light output, during which time mercury droplets in the lamp evaporate and form excess mercury vapor which condenses onto the coldest spot in the lamp until equilibrium is reached between the mercury vapor pressure and the condensed mercury at the "cold spot." A typical size of the cold spot is about one-eighth to one-fourth of an inch in diameter. A desirable temperature of the cold spot is 40° C, causing a mercury vapor pressure in the lamp of about 6 microns, which causes maximum light to be produced by the phosphor in the lamp. A certain amount of condensed mercury is desirable in the lamp to insure against depletion of mercury, and hence reduction of mercury vapor pressure, during the life of the lamp.

FIG. 1 of the drawing is derived from FIG. 2 of "Light Output of 1.5 Ampere Fluorescent Lamp Designs in Photometry and Use" by Beck, Gabriel and Aicher, on pages 167-175 of "Illuminating Engineering," Vol. LXIII, No. 4, April 1968. It shows that, during initial operation of a T12 fluorescent lamp at 1.5 amperes (solid-line curve) the light output is reduced to 85 percent of its final value for nearly fifty hours, until mercury stabilization occurs. The dashed line shows the light output for subsequent restarts in which the condensed mercury remains at the cold spot of the lamp and hence no substantial amount of time is required for further stabilization.

The location of the "cold spot" of the lamp, at which the mercury vapor condenses, depends on lamp design. In a long lamp have short lamp mounts, the cold spot will be at the center of the lamp bulb. The cold spot will be at an end of the lamp bulb if the lamp mount at that end is made long enough. Further details of lamp design and cold spot locations are described in "External Control of Mercury Pressure of Fluorescent Lamps and Its Application to Luminaires" by Underwood and Beck, a six-page published paper presented at the National Technical Conference of the Illuminating Engineering Society, Sept 7-11, 1959, in San Francisco, Calif. This paper also describes external control and cooling of the cold spot by means of cooling fins, air jets, and other devices, when a lamp is operated in a high ambient temperature or at increased current and hence increased temperature, the purpose of such external cooling being to maintain the cold spot at optimum operating temperature during operating life of the lamp so as to insure optimum mercury vapor pressure and light output.

Now referring again to FIG. 1 of the drawing, it will be evident that the many hours of reduced light output during initial operation of a mercury-vapor lamp, caused by the mercury stabilization process just described, is particularly undesirable in certain applications. For example, document copying machines such as xerographic machines utilize a mercury-vapor fluo-

rescent lamp to scan and/or illuminate the document to be copied, and the quality of the copies is dependent on the brightness of the lamp. The reproduced copies are of inferior quality when made during the initial hours of lamp operation and stabilization. Of course, the lamp may be operated during the initial stabilizing period in an idle machine, which is costly and time-consuming. Operating the lamps at the factory or elsewhere until mercury stabilization is achieved, also is costly and time-consuming, and is not often successful because subsequent shipping or handling is likely to cause the condensed mercury to leave the cold spot and roll to other places in the lamp, whereupon the low light output stabilization period will again occur in whole or in part.

From the foregoing, the need is apparent for a method of stabilizing, or prestabilizing, mercury vapor lamps quickly and permanently.

### SUMMARY OF THE INVENTION

Objects of the invention are to provide an improved method of stabilizing mercury vapor lamps, and to provide a method of prestabilizing mercury vapor lamps relatively quickly and permanently.

The invention comprises, briefly and in a preferred embodiment, prestabilizing a mercury-vapor lamp by temporarily operating the lamp while at the same time cooling a small area of the lamp bulb, at the normal "cold spot" location where the mercury will normally condense during lamp operation to a temperature lower than its normal intended operating temperature. This method causes the mercury to condense quickly (typically in 1 to 2 hours) at the cold spot, and the method also advantageously causes the mercury to adhere to the phosphor and the bulb at the cold spot. The lamp may then be shipped and put into use and, due to the aforesaid prestabilization, the lamp will quickly operate at full normal brightness without the need for any appreciable further stabilization time period. The cooling of the cold spot may be achieved by an air jet, cooling fins, or other convenient means. If the lamp has a reflector coating between the bulb and the phosphor coating, as is the case with a typical reprographic lamp, preferably the reflector coating is removed or deleted at the area of the cold spot, so that during the prestabilization the mercury can more readily penetrate the phosphor and come into contact with the glass bulb (or with a precoat on the bulb if such is employed). A layer of indium, sodium sulfate, or other mercury-wettable material at the cold spot, preferably between the phosphor layer and the bulb, improves adhesion and entrapment of the mercury at the cold spot. Also, making the phosphor layer thicker, and/or of coarser or larger granules at the cold spot area, improves adhesion and entrapment of the mercury so that it will be less likely to become dislodged during subsequent handling, shipping, and installation in equipment.

### BRIEF DESCRIPTION OF THE DRAWING

FIG. 1 is a plot of curves showing the prior art stabilization and operating characteristics of mercury-vapor lamps;

FIG. 2 is a side view of a mercury vapor fluorescent reprographic lamp in the process of being prestabilized in accordance with a preferred embodiment of the invention;

FIG. 3 is a cross-sectional view taken on the line 3—3 of FIG. 2, on an enlarged scale; and

FIG. 4 is a set of curves illustrating the prestabilization and operating characteristics of lamps processed in accordance with the invention.

#### DESCRIPTION OF THE PREFERRED EMBODIMENT

To better facilitate understanding of the invention, mercury stabilization characteristics of prior art lamps will now be described, with reference to FIG. 1. In FIG. 1, the vertical axis 11 represents relative light output of a mercury vapor fluorescent lamp, and the horizontal axis 12 represents operating time of the lamp, this time axis being separated, for clarity, into a first-part operating time of 0 to 20 minutes, and a subsequent continuing operating time of from 2 to 250 hours. The solid-line curve 13 represents light output with respect to initial operating time of a T12 fluorescent lamp operating at 1.5 amperes, and the dashed-line curve 14 represents the same lamp when operated subsequently provided that the lamp has not been jostled so as to dislodge the mercury that has condensed at the cold spot of the lamp. When a lamp is initially operated, its light output exceeds the normal 100 percent light output by about 10 percent for a minute or two, as shown by curve 13 in FIG. 1 (during this period, the lamp is warming up and the mercury vapor pressure is increasing through its optimum pressure of 6 microns, and then considerably exceeds this pressure), and then the light output of the lamp reduces to about 85 percent of its final operating value and continues at this decreased light output value for a considerable number of hours, for example up to 50 or more hours, while excess mercury vapor in the lamp is traveling toward and condensing at the cold spot of the lamp. When all of the excess mercury vapor in the lamp has condensed at the cold spot, mercury vapor equilibrium is reached and the mercury vapor pressure in the lamp is a function of the temperature of the cold spot. Preferably, the cold spot is about 40°C, which causes the mercury vapor pressure in the lamp to be about 6 microns, which is optimum vapor pressure for causing the 100 percent relative light output of the lamp.

If the lamp remains in position and is not jostled, the condensed mercury remains collected at the cold spot of the lamp after the lamp is turned off, and when the lamp is subsequently turned on, its brightness output follows the dashed-line curve 14 and the light quickly assumes its normal 100 percent light output since no further mercury stabilization is required. If, however, the lamp is jostled or shipped from one location to another, or removed from a fixture or equipment and reinserted, the condensed mercury globule is likely to become dislodged, and mercury will roll around and scatter within the bulb, whereupon subsequent operation of the lamp requires a repeat of some or all of the hours of stabilization time.

In the embodiment of the invention shown in FIG. 2, a mercury vapor reprographic fluorescent lamp 16 comprises an elongated soda lime silica glass tube 17 of circular cross-section. The lamp is provided with the usual electrodes 18, 19 at each end thereof, respectively supported by inlead wires carried in stems 21, 22 of glass which are respectively sealed to the two ends of the envelope tubing 17. Bases 23, 24 of conventional design are attached to the ends of the glass envelope

17. As shown, one of the glass stems 22 is longer than the other, so that during operation of the lamp the end of the envelope 17 at which the longer stem 22 is located, will be the relatively coldest part of the lamp. 5 During manufacture, various layers of material are coated inside the envelope tubing 17, as will be described, and then the lamp is processed and filled with an inert gas such as argon or a mixture of argon and neon, at suitable pressure, and also is provided with a 10 small quantity of mercury, at least enough to provide a low vapor pressure of about 6 microns during operation of the lamp under normal operating conditions.

As best shown in FIG. 3, the inner surface of the glass envelope 17 is protectively coated with a thin, clear 15 film 26 consisting of titanium dioxide. In one way of forming this layer, a metallo-organic compound of titanium such as tetrabutyl titanate or tetraisopropyl titanate dissolved in an appropriate solvent such as butyl alcohol or butyl acetate, is applied to the glass. The solvent evaporates quickly and the titanate is left deposited upon the inner surface of the glass tube. Moisture from the air hydrolyzes the titanate almost as fast as the solvent evaporates, forming titanium dioxide which remains as a very thin clear continuous film in a thickness 20 from 0.002 to 0.02 microns.

25 The lamp then is provided with a reflector coating 27, which may be a particulate coating of titanium dioxide having a particle size less than 1 micron, for instance centering on about 0.3 micron which is about 30 half the median wavelength of the visible spectrum. The titanium dioxide ( $TiO_2$ ) may be applied as a suspension in a solution of ethyl cellulose in an organic solvent to serve as a binder, the suspension being drawn up into the tube while supported vertically and then allowed to drain out. Thereafter the tube is lehred in order to decompose and drive out the organic binder. Alternatively, the reflector coating may consist of magnesium oxide ( $MgO$ ). A phosphor coating 28 is applied over the inside surface of the reflector coating 27, and 35 may consist of calcium halophosphate, applied as a suspension in a solution of nitrocellulose in butyl acetate which is drawn up into the tube and allowed to drain out.

40 A transparent aperture 29 is then formed along the 45 side of the lamp, by scraping away the reflector and phosphor coatings over an area to form the elongated clear window or aperture 29, as shown. The clear protective layer 26, however, remains since it is extremely 50 adherent to the glass envelope 17. Instead of scraping material away to provide the aperture 29, it may be formed by applying the reflector and phosphor coating materials, in succession, into the tubing while supported horizontally and rocked back and forth about its 55 elongated axis to coat the bulb only over the desired area, as taught in U.S. Pat. No. 2,892,440 — Fulton et al.

60 Prior to applying the phosphor layer in the lamp as has been described, a small area of the reflector 27 may be removed at the "cold spot" location in the lamp, which, in the lamp illustrated, is near the end of the envelope at which the longer stem 22 is sealed, and at the 65 side of the lamp away from the aperture window 29, as indicated by the numeral 31 in FIG. 3. The size of the scraped-away reflector material at 31 may be approximately one-eighth to one-fourth of an inch diameter, or a square shape approximately one-eighth to one-fourth inch on the side, or any other easily scraped-away

shape of the same general size or larger. Alternatively, the same result may be achieved by not coating the cold spot region. The layer of phosphor 28, when subsequently applied, fills in the cleared-away area at 31, as shown in FIG. 3. Alternatively to the foregoing procedure, the phosphor layer 28 is applied over the reflector and then both the phosphor and reflective material 27 are scraped away at the area 31, whereupon additional phosphor or other mercury-absorbing material is applied in the area thus scraped away. In a modification of the invention, before phosphor is applied at the area 31, a layer of mercury-wettable material 32, such as indium or sodium sulfate, is applied to the envelope tubing 17, or to the protective coating 26, at the area 31, and then a layer of phosphor 28 is coated over the inner surface of this mercury-wettable material.

After the lamp 16 is assembled, and filled with gas and dosed with mercury, all as described above, and sealed off and with the bases 23, 24 either attached or not yet attached, and in accordance with the invention, the lamp is prestabilized as follows. The lamp is operated temporarily, preferably with normal operating current, while at the same time the cold spot area 31 is cooled by external means, such as by an air jet, cooling fins, or other suitable means, to a temperature lower than its normal intended operating temperature. The drawing shows a cooling fin arrangement 36 comprising a cooling block 37 provided with radiation fins 38, and shaped to fit the outer contour of the envelope tubing 17 at the cold spot area 31, and held in place by means of a pair of spring-wire clips 41, 42 which partially encircle the outer periphery of the tubing 17 in a gripping relationship thereto. The lamp is thus operated with external cooling of the cold spot area 31 until the excess mercury vapor in the lamp has migrated toward and condensed at the cold spot area 31. It is found that this procedure stabilizes the lamp much more quickly than would occur in normal operation, and it has been further found that this procedure provides the very beneficial result of sufficiently adhering the condensed mercury globule 46 at the cold spot region, so that the lamp may subsequently be handled, shipped, and installed in equipment, with considerable likelihood that the mercury globule 46 will remain in position at the cold spot area 31, whereupon the lamp will be immediately usable at full normal brightness, without having to undergo a time period of reduced brightness while mercury stabilization occurs.

FIG. 4 is a plot of curves, generally similar to FIG. 1, showing the quick prestabilization of the mercury achieved by the invention. In FIG. 4, the vertical axis 48 represents relative light output and the horizontal axis 49 represents lamp operating time. The scale of relative light output on the vertical axis 48 is the same as that of vertical axis 11 in FIG. 1; however, as will be readily seen, the time scale of the lamp operating time horizontal axis 49 is considerably shortened with respect to that of lamp operating time axis 12 of FIG. 1. In FIG. 4, the solid-line curve 51 represents the light output of the lamp 16 (which, in this case, is a T12 lamp operated at 1.5 amperes, the same as that used to obtain the curves in FIG. 1) during the prestabilization process. As shown, during prestabilization the lamp operates at a low output light level of about 85 percent of normal 100 percent light output, for a period of only 1 to 2 hours, whereupon the excess mercury vapor pressure has condensed into the globule 46 at the cold spot

of the lamp. The external cooling means 36 is then removed; if left on the lamp, the mercury vapor pressure would be less than optimum and the light output would be reduced. Thereafter the cold spot 31 is at its normal intended operating temperature and the lamp operates at normal 100 percent light output. In subsequent lamp operation, such as when the lamp has been shipped and installed in equipment, the light output assumes that of the dashed line curve 52, i.e., the lamp assumes normal 100 percent light output immediately after a short one or two minute period of slightly increased light output. Thus, no time need be wasted, after the lamp is installed in equipment, for stabilizing the mercury. This achievement is due to the fact that, in accordance with a feature of the invention the prestabilization of mercury as described above causes the mercury to adhere to and remain at the cold spot area of the lamp, during handling and shipping and installation, so there is no substantial amount of loose mercury elsewhere in the lamp that must be stabilized into the cold spot area during operation of the lamp.

It has been found that only a slight amount of external cooling of the cold spot region of the lamp, to render the cold spot slightly colder than its normal intended operating temperature during the prestabilization process, is sufficient to achieve quick condensation and firm adherence of the excess mercury in the lamp at the cold spot region 31. It has further been found that external cooling of the cold spot region 31 to a considerably lower temperature, such as by applying dry ice externally to this cold spot region 31, quickens the prestabilization somewhat, but at greater expense and inconvenience, and therefore the cooling fin technique described above is a preferred method of externally cooling the cold spot area 31. For a lamp designed to operate with an optimum cold spot temperature of 40° C, external cooling to reduce the cold spot temperature to about 30° C or 35° C during the prestabilization, produces satisfactory results. The prestabilization time period can be shortened somewhat by operating the lamp at increased operating current, and hence increased operating temperature, during the prestabilization period.

It is believed that the prestabilization in accordance with the invention causes the mercury to be absorbed and trapped into the phosphor 28 and/or adhered to the glass surface, or protective coating, or mercury-wettable coating 32, for reasons not fully understood at present. Perhaps the temperature gradient produced by the spot-cooling causes the mercury to be "pulled" through the phosphor and/or  $TiO_2$  or other coating materials, toward the glass bulb. The process should also be useful for other metallic-vapor discharge lamps.

The invention has been particularly described in connection with a mercury-vapor fluorescent reprographic lamp; however, the invention also can be utilized with beneficial results on other types of fluorescent and mercury-vapor lamps.

In applying the invention to prestabilization of high-temperature lamps intended to be operated with cooling fins or other cooling means at the cold spot (for maintaining the cold spot at optimum temperature such as 40° C), the prestabilization is achieved by "super cooling" the cold spot to reduce its temperature to a value lower than the intended operating temperature. This can be achieved by using larger cooling fins, or

with forced-air cooling of the fins, or dry ice, for example.

While preferred embodiments and modifications of the invention have been shown and described, various other embodiments and modifications thereof will be apparent to those skilled in the art, and will fall within the scope of invention as defined in the following claims.

What we claim as new and desire to secure by letters Patent of the United States is:

1. A method of prestabilizing, prior to use thereof, a metallic-vapor reprographic lamp of the type having a cylindrical bulb and containing a coating of reflector material within the bulb, the reflector material being coated interiorly at least in part with phosphor material, said lamp being designed so that during normal operation thereof excess metallic vapor material condenses at a cold spot region located at said reflector and phosphor coatings, said method comprising the steps of providing an opening through said reflector coating at said cold spot region whereby said phosphor extends into said opening toward said bulb, temporarily operating said lamp and simultaneously temporarily ap-

plying cooling means for cooling said cold spot region to a temperature lower than the intended normal operating temperature thereof for a time sufficient to cause a desired amount of the metallic vapor material to condense at said cold spot region, and removing said cooling means so that in subsequent lamp operation said cold spot region will be at said normal operating temperature.

2. A method as claimed in claim 1, in which said time of prestabilization operation and cooling is sufficiently long to cause substantially all excess metallic vapor material in the lamp to condense at said cold spot region.

3. A method as claimed in claim 1, in which said cold spot region is temporarily cooled to a temperature several degrees Centigrade lower than the normal intended operating temperature thereof.

4. A method as claimed in claim 1, in which said metallic vapor is mercury.

5. A method as claimed in claim 1, in which said cooling means is a cooling fin means applied against said lamp at the region of said cold spot.

\* \* \* \* \*

25

30

35

40

45

50

55

60

65